

Oct. 17, 1972

B. GIBERSTEIN  
METHOD OF MANUFACTURE OF PRINTED ARTICLES, IN  
PARTICULAR PRINTED KNITTED ARTICLES  
Filed Aug. 17, 1970

3,698,899



INVENTOR  
BERNARD GIBERSTEIN

BY

Nolte & Nolte  
ATTORNEYS

**1**

3,698,899

**METHOD OF MANUFACTURE OF PRINTED ARTICLES, IN PARTICULAR PRINTED KNITTED ARTICLES**

Bernard Giberstein, Paris, France, assignor to Bégy Société Européenne de Bas sans Couture, Autun (Saône-et-Loire), France  
Filed Aug. 17, 1970, Ser. No. 64,428  
Claims priority, application France, Aug. 27, 1969,  
6929321; June 10, 1970, 7021298  
Int. Cl. G03c 5/04

U.S. CL. 96—27

5 Claims

**ABSTRACT OF THE DISCLOSURE**

A method of manufacture of printed knitted articles, hosiery, stockings, tights and the like wherein, in order to carry out the desired printing, the article is provided with a light sensitive substance at a given moment during its treatment, it is fitted on a form and subsequently subjected to photographic exposure which acts upon the said substance, and the said exposed substance is thereafter developed and fixed on the said article.

The present invention has essentially for its object a method of manufacture of printed textile articles and especially knitted goods and hosiery, in particular thin stockings and tights or skin-fitting garments for women.

Textile articles are known which are provided with printed patterns or designs. Such printed articles are usually connected with small-scale production.

Where the articles, such as scarves, have a flat shape, the printing may be performed more or less in series, by using for instance such techniques as serigraphy.

On the contrary, where shaped articles are concerned, no convenient industrial or even semi-industrial process is known. Under such conditions, it is necessary to result to small-scale production using series which are necessarily very limited. Under such conditions, except where the design or pattern is not extremely simple, production costs rapidly become prohibitive.

If in order to avoid this difficulty the impression is effected on the shaped article in the flattened state, there necessarily appears connections which are detrimental to the harmony of the finished products and which, on the other hand, compel to take numerous precautions for preventing the colour of one printed portion from coming off on another during manufacture.

The invention has for its object to enable the manufacture of printed articles and in particular shaped knitted articles and hosiery, especially thin stockings and tights for skin fitting garments for women, the method of the invention enabling if desired, to effect the printing on an industrial scale at corresponding costs.

The method according to the invention uses a printed textile article manufacturing process wherein the desired printing is obtained by providing the article with a photo-sensitive substance at a given moment during its treatment, subjecting it subsequently to a photographic exposure which acts on the said substance, and thereafter developing and fixing the said exposed substance on the said article. Methods of this type were known in the prior art and used for photographic printing of fabrics laid flat.

According to the invention the method is characterized in that in being applied to shaped or non-shaped articles such as knitted articles and hosiery, especially thin stockings and tights for women, the said photographic exposure is carried out while the article is fitted on a form with the entire inside surface of the tubular garment continuously contacts the inserted tubular form.

The photographic exposure may be performed for in-

**2**

stance on a form bearing the pattern to be reproduced and illuminated during the exposure, for instance from the inside, and during an appropriate period of time by means of a radiation source to which the said photosensitive substance is sensitive.

It is thus understood that if, for instance, a mode of photographic reproduction of the "negative" "positive" type is used with a form bearing the "negative" pattern or design which it is desired to transfer onto the article, 10 it is possible to manufacture the required number of articles displaying the corresponding "positive" pattern subsequent to photographic exposure, development and fixation.

Indeed, it is sufficient to simply fit every time the article onto its form, and then to effect the photographic exposure, the same form being used as many times as desired for other articles to be manufactured.

Subsequent to manufacture of the desired quantity of articles in a given series, it is possible to destroy the form, 20 thus limiting the exclusive printing of a pattern to a desired quantity.

The photosensitive substance which enables to transfer the design or pattern onto the form may be constituted in various manners.

25 It may for instance be constituted in the form of a more or less conventional photographic emulsion which is applied on the article and maintained there in any appropriate manner. The emulsion may be applied for instance by way of coating or impregnation. The photo-sensitive substance may be included in a solution, paste or paint. The fixation on the article, for instance on a nylon stocking or tights, may be obtained by using a glue or adhesive or finish according to the methods known in the manufacture of dyed or printed textile articles.

30 Alternatively, the photosensitive substance may be included in the textile material itself, for instance in the fibres constituting the same. The fibres may be provided with coloured pigments which will cause their colour to change when the fibres are suitably exposed.

40 The photographic printing may be effected by means of any suitable radiation to which the photosensitive substance used is sensitive. Infra-red (heating), visible (according to conventional photographic techniques) or ultra-violet (according to the conventional techniques used in the printing of drawings) may be used. X or  $\gamma$  radiation may also be used.

45 The photographic exposure may be effected simply, as already stated in the foregoing, by fitting the article onto a form bearing the design or pattern to be reproduced and illuminated from the inside by means of a source of sensitizing radiation. For instance, the form may be made from transparent or translucent plastics on which the positive or negative design to be reproduced are drawn.

50 In the case of printing in several colours, the method may be carried out by using several forms and the design reproduced on the article from each form may correspond to a given colour. The photographic printing may also be carried out from the outside instead of the inside of the form. For instance, the article may be fitted onto the form and the latter while turning on itself may be subjected to the light beam of an image which may possibly change or pass along. Alternatively, the form may be stationary and the image may be projected on the form all around the latter, either by means of a convergent cylindrical beam or by means of a light beam moving round the form.

55 The invention also relates to improvements in the devices enabling to carry out the method in an economical and practical manner. It will appear more clearly from the following description made with reference to the appended drawings illustrating by way of example a few

forms of embodiment of the invention as applied to the manufacture of stockings. In the said drawings:

FIG. 1 diagrammatically illustrates the sequence of successive operations used in carrying out the method of the invention;

FIG. 2 is a longitudinal sectional view illustrating diagrammatically and to a larger scale one of the steps of the manufacturing process illustrated in FIG. 1;

FIG. 3 is a top view of FIG. 2;

FIG. 4 is a perspective view of a form which may be used in carrying out the photographic printing according to the invention;

FIG. 5 diagrammatically illustrates an alternative process of photographic exposure of the article fitted onto a form according to the method of the invention;

FIG. 6 is a view similar to that of FIG. 2 illustrating a further alternative process of photographic exposure of an article fitted onto a form according to the invention.

Reference is first made to FIG. 1 illustrating a succession of operations enabling to carry out the photographic printing, for instance on stockings.

The stockings **10** falling from the knitting machine and not yet sewn at their ends are emerged into a dye bath **11** containing the sensitive material enabling the photographic printing of the stocking. When this stage **1** of the dying of the stocking is completed, the dyed stocking **12** is conveyed to a cylindrical form **13** and fitted onto it. These operations are numbered **2** and **3** in FIG. 1.

The dyed stocking impregnated with sensitive material and fitted onto its form **13** is thereafter subjected to photographic exposure during the fourth stage of the process. This stage is denoted by the numeral **4** in FIG. 1. As appears more clearly from FIGS. 2 and 3, the form **13** is illuminated from the inside by luminescent tubes **14** and it rotates on the plate **25** driven by a roller **26** mounted on the shaft **27** of an electric motor **28**.

As appears in FIG. 4, the form **13** bears designs or patterns **19** on its external surfaces. The form may be constituted by a cylinder made from transparent or translucent plastics or from any other equivalent or suitable material, and it may be decorated externally, internally or in its mass by any method leaving its imprint, so that during illumination from the inside by means of the tubes **14**, the stocking **12** is subjected to the photographic exposure of an image. Thus, owing to the impregnation of the stocking **12** with a light sensitive material, there is formed on the stocking a latent image which it is thereafter sufficient to develop and fix.

Advantageously and simultaneously with this photographic exposure stage a drying operation is carried out by making hot air circulate as diagrammatised by the arrows **f**, in order to dry the stocking **12** on its form **13**.

Subsequent to photographic exposure, the stocking **15** having a latent image and partially dried is stored on the form **13** in an atmosphere which enables to disclose the image. According to a method which will be described later, the atmosphere is basic, for instance ammoniacal. This developing and disclosing stage is denoted at **5** in FIG. 1.

Subsequent to disclosure of the image, the latter is fixed on the fabric. This is the fixing operation denoted at **6** in FIG. 1. The fixation is advantageously effected on the form, for instance by means of steam, under pressure or not. The steam causes the dye stuffs to penetrate into the fabric.

Subsequent to fixation of the image, the articles **17** are withdrawn from the form **13** and carefully washed in a bath **18** as illustrated at **7** in FIG. 1.

Examples of printing of stockings according to this method will now be described.

#### EXAMPLE 1

The knitted stockings made from nylon or the like, proceeding from the knitting machine and the end of

which is not yet sewn, are decreased in the usual manner so as to provide an article having a white background.

In the last rinsing bath, a light sensitive material is introduced, which is constituted in the following manner:

- 5 from 3 to 10 g. per litre of a diazo dye salt such as "diazo salt" marketed by the firm Francolor from 1 to 3 g. per litre of resorcin
- 10 from 3 to 10 g. per litre of tartaric acid
- 10 g. per litre of glycerin ensuring the penetration and dispersion of the products in the emulsion
- 10 g. per litre of a finish or an emulsion such as lanolin emulsion forming a thickening agent, selected for instance among the products sold by Société Ciba and known under the denomination "Sapamine" (registered trademark).

Subsequent to impregnation of the article with the sensitive solution, followed by squeezing, pressing out or centrifuging, the article is fitted onto the form **13** as diagrammatised at **3** in FIG. 1.

The article is thereafter subjected to photographic exposure during the required time depending on the concentration of sensitive material, the light energy used and the nature of the image borne by the form.

- 25 In those areas where the light reaches the stocking, the dye stuff is destroyed and subsequent to development the areas exposed to light appear in white.

Subsequent to photographic exposure and suitable partial drying, the article is stored on its form in an ammonia gas atmosphere which develops the dye-stuff in all the areas where it has not been destroyed by the light. In the example described where use is made of resorcin, the stocking areas which have been protected from light appear in chestnut colour.

35 Subsequent to suitable development, and while the stocking is still on its form, it is subjected to a steam bath, under pressure or not. The steam causes the dye-stuff to penetrate into the fabric thus fixing the image on the stocking in an indelible manner.

40 Subsequent to fixation of the image, the stocking is suitably rinsed so as to be freed from the residual products which have not reacted.

#### EXAMPLE 2

45 The same process as in Example 1 is applied, except that a pyrazolin salt is used instead of resorcin. In this case, the image which may be called "positive" since it appears there where the light has not reached the stocking, appears in red on a white background and not in chestnut colour on a white background.

#### EXAMPLE 3

The same process is applied as in Examples 1 and 2, except that phloroglucin is used instead of resorcin. The 55 image this time appears in grey on a white background.

#### EXAMPLE 4

The same process is applied as in Examples 1, 2 or 3, except that instead of degreasing or in addition to degreasing, the stocking proceeding from the knitting machine is dyed.

In this case, the impregnation with sensitive material may be carried out simultaneously with the dyeing or subsequent to dyeing.

65 In this case, the positive image formed appears on a coloured background and not on a white background as previously.

#### EXAMPLE 5

70 The same process is applied as in the preceding examples, except that the sensitive material is replaced by a dyestuff of the type known under the trademark "Indigosol" supplied by the Sandoz laboratories or "Solasol" supplied by the Francolor laboratories. In this case, the 75 printing obtained is a negative printing, i.e. the image

subsequent to development appears coloured in the areas where the light has not reached the stocking.

If it is desired to obtain designs or pattern in several colours and more complicated, several successive operations may be carried out, and, in particular, a positive printing and a negative printing may be combined to obtain quite varied designs.

In the alternative embodiment illustrated in FIG. 5, the photographic exposure of a stocking 20 fitted onto a cylindrical form 21 is effected not from the inside but from the outside by means of a projector 22 rotating about the stocking and illuminating it by a light beam 23. Any desired image may thus be projected on the stocking. Alternatively, the form 21 may be made to rotate about its axis, the projector 22 remaining stationary.

In the alternative embodiment diagrammatized in FIG. 6, the illumination of a form 29 is effected from the inside by means of a projector 24 which may be constituted for instance by an electronic flash. A reflector 30 mounted in the lower portion of the form 29 reflects the light provided by the flash.

This arrangement offers a certain number of advantages as compared to the form of embodiment illustrated in FIG. 2. In particular, it is not necessary in this case to cause the form to rotate on itself and it is not necessary to place the form 13 around the tube 14, since the flask 24 may be positioned in any convenient place above the form 29. It is not necessary either that an electric supply wire 39 should pass through the tube 14 (FIG. 2). In addition, it is easier to adjust very accurately the light energy from the flash 24 and therefore to obtain more accurate and uniform results.

Of course, the invention is by no means limited to the forms of embodiment described and illustrated, which have been given by way of example only, and the invention comprises all the technical means equivalent to those described as well as their combinations, if the latter are carried out according to its spirit within the scope of the following claims.

What is claimed is:

1. A method of photoprinting on a continuously tubular knitted garment element, comprising: impregnating said garment element with light-sensitive substance opening a tubular section in said element and coaxially mounting it on, coaxially tubular form with the entire inside

surface of the tubular garment element continuously contacting said form, photographically projecting a peripherally continuous design onto said light-sensitive impregnating substance in the tubular garment element which contacts the form, axially removing the garment element from the form, and developing and fixing the projected design on the garment element.

2. A method of photoprinting according to claim 1, wherein the light sensitive substance is applied to the garment in the form of a coating.

3. A method of photoprinting according to claim 1, wherein the light sensitive substance constitutes an ingredient forming part of the knitted garment.

4. A method of manufacture according to claim 1, wherein the impregnating is performed in a dye bath.

5. In the process of claim 1, wherein the tubular form is translucent and carries a design to be reproduced on the garment element.

#### References Cited

#### UNITED STATES PATENTS

|           |         |                  |       |         |
|-----------|---------|------------------|-------|---------|
| 2,653,529 | 9/1953  | Stover           | ----- | 355—104 |
| 2,985,502 | 5/1961  | Kronsbein et al. | ----- | 8—150   |
| 2,875,677 | 3/1959  | Ellis            | ----- | 240—49  |
| 2,743,653 | 5/1956  | Kennedy et al.   | ----- | 355—104 |
| 3,221,597 | 12/1965 | Vogt             | ----- | 98—24   |
| 3,191,182 | 6/1965  | Caldwell et al.  | ----- | 95—16   |
| 2,980,534 | 4/1961  | Printy et al.    | ----- | 96—49   |
| 2,549,546 | 4/1951  | Thomas           | ----- | 355—3   |
| 2,464,793 | 3/1949  | Cooke            | ----- | 95—15   |
| 1,972,323 | 9/1934  | Shirreff et al.  | ----- | 96—49   |
| 1,943,377 | 1/1934  | Ellis            | ----- | 8—2     |
| 1,841,653 | 1/1932  | Grinters et al.  | ----- | 96—49   |
| 1,751,774 | 3/1930  | Trullinger       | ----- | 95—15   |
| 1,669,826 | 2/1928  | Winogradoff      | ----- | 8—2     |
| 1,618,931 | 2/1927  | Kammerer         | ----- | 96—49   |
| 875,770   | 1/1908  | Borzykowski      | ----- | 8—2     |
| 306,481   | 10/1884 | Gottlier         | ----- | 96—49   |
| 241,713   | 5/1881  | Pellet           | ----- | 96—49   |
| 40        | 656,015 | Dommer           | ----- | 8—2     |
|           | 8/1900  |                  |       |         |

DONALD LEVY, Primary Examiner

U.S. Cl. X.R.

45 8—2; 95—1